

April 23, 1935.

A. VON BIEHLER

1,998,530

PHOTOGRAPHIC MATERIAL

Filed Aug. 4, 1931



Inventor:

Arpad von Biehler,  
By Attorney Philip S. Hopkins.

## UNITED STATES PATENT OFFICE

1,998,530

## PHOTOGRAPHIC MATERIAL

Arpad von Biebler, Dessau in Anhalt, Germany,  
assignor to Agfa Ansco Corporation, Binghamton, N. Y., a corporation of New York

Application August 4, 1931, Serial No. 555,080  
In Germany August 8, 1930

7 Claims. (Cl. 95—2)

My present invention relates to light-sensitive photographic materials and more particularly to such materials as used, for instance, in color photography.

5 One of its objects is to provide photographic materials bearing on their light-sensitive emulsion layer a colored filter layer.

Further objects of the invention will be seen from the detailed specification following here-  
10 after, reference being made to the accompanying drawing showing in cross section in an enlarged scale a photographic film made according to the invention.

Processes are known for providing light-sensi-  
15 tive photographic layers, which are intended for the preparation of negatives on which the individual color sensations are registered, on their surfaces with filter layers, so that only light of fixed wave lengths can act upon the underlying layer of the light-sensitive material. Water-  
20 soluble dyes are used for this purpose, since the dye has to be removed by the photographic treating liquids, in order that it may not interfere with the printing operation. When using, how-  
25 ever, water-soluble dyes, the dye diffuses into the emulsion layer during prolonged storage of the photographic material, owing to the natural mois-  
ture content of the layer, and this may detri-  
30 mentally effect the sensitiveness of the emulsion layer. If, for instance, in a three-pack process a yellow filter layer is arranged behind a layer  
35 sensitive to blue light, the sensitiveness is con-  
siderably reduced, by diffusion of the yellow dye into the emulsion layer sensitive to blue light.

According to my present invention, this draw-  
35 back is avoided by coating the surface of the emulsion layer with a layer containing a water-  
insoluble dye, which is decolorized or rendered water-soluble by the action of the photographic  
40 treating liquids or by a special after-treatment. The filter layer may likewise be made of a water-  
insoluble colloid which is destroyed or rendered soluble in the photographic treating liquids or by a special after-treatment.

45 For the dye layer applied to the surface of the emulsion layer there are especially suitable those water-insoluble dyes which are soluble in organic solvents, and preferably those which, owing to the presence of acid or hydroxyl groups, are ca-  
50 pable of forming water-soluble alkali salts. If the filter is made up of a colloid layer, the colloid being insoluble in water but soluble in the photo-  
graphic liquids or a special after-treatment bath, and being preferably soluble in organic sol-  
55 vents, any dyes, water-insoluble as well as water

soluble dyes may be incorporated in this colloid layer. As a colloid of the kind described I may use abietic acid which is very well suited, but other colloids such as nitro-cellulose and acetyl-cellulose, preferably when made into very thin layers are likewise suitable. There may also be used water-insoluble dyes combined with water-  
insoluble colloids which are soluble in organic solvents and can be destroyed by a suitable after-treatment.

10 There can be used for the coloration, of course, also mixtures of dyes, or dyes and colloids having the properties required. The layers can be colored, for instance, by coating, spraying or dipping processes.

15 The following examples illustrate the invention.  
Example 1.—A silver bromide gelatin layer is colored on the surface with a 10% alcoholic solution of water-insoluble Aurine (cf. Schultz, Farbstofftabellen, 6th edition, No. 555).

20 The dye is rendered water-soluble by the treatment in the photographic developer and fixing bath and, therefore, washed out.

25 In the foregoing example the water-insoluble Aurine may be substituted, for instance, by Resoflavine W (771), Alizarine-black WR (774), Purpurine (783), Cyanosine (soluble in alcohol) (594) and Gallocyanine (626). The numbers given relate to Schultz, Farbstofftabellen, 6th edition.

30 Instead of Acridine orange there may be used Uranine (cf. Schultz, Farbstofftabellen, 6th edition, No. 585). The collodion solution may be replaced by a 0.1% solution of cellulose acetate.

35 Example 2.—A silver bromide gelatin layer is coated with a thin layer of a 5% alcoholic abietic acid. Then a mixture of equal parts of a 10% alcoholic solution of abietic acid and of a 1% solution of Violamine R soluble in alcohol (color acid, cf. Schultz, Farbstofftabellen, 6th edition, No. 582), in alcohol is applied thereto. Before the development the dye is eliminated by a treatment in a sodium hydroxide solution of 1/2% strength.

40 In the accompanying drawing A is a support for the light-sensitive emulsion B, which either is colored by a water-insoluble dye or which may bear a further layer C (indicated in the drawing by dotted lines), in which the water-insoluble dye is incorporated.

45 My invention is not limited to the foregoing examples or to the specific details given therein. Numerous other dyes and colloids are suitable the qualification of which can easily be determined by a few simple experiments.

What I claim is:—

1. With a photographic material comprising a support provided with a light-sensitive emulsion, a color filter applied to the surface of said emulsion layer, said filter consisting of a mixture of a dye and a colloid which is insoluble in water but soluble in the photographic treating baths. 5
2. With a photographic material comprising a support provided with a light-sensitive emulsion, a color filter applied to the surface of said emulsion layer, said filter consisting of a mixture of a dye and a colloid which is insoluble in water but soluble in the photographic treating baths and in organic salts. 10
3. With a photographic material comprising a support provided with a light-sensitive emulsion, a color filter applied to the surface of said emulsion layer, said filter consisting of a mixture of a dye and a colloid both being insoluble in water but soluble in the photographic treating liquids and in organic solvents. 15
4. With a photographic material comprising a support provided with a light-sensitive emulsion, a color filter applied to the surface of said emulsion layer, said filter comprising a dye which is insoluble in water but soluble in the photographic treating baths. 5
5. With a photographic material comprising a support provided with a light-sensitive emulsion, a color filter applied to the surface of said emulsion layer, said filter consisting of water insoluble 10 aurine.
6. With a photographic material comprising a support provided with a light-sensitive emulsion, a color filter applied to the surface of said emulsion layer, said filter consisting of gallocyanine. 15
7. With a photographic material comprising a support provided with a light-sensitive emulsion, a color filter applied to the surface of said emulsion layer, said filter consisting of abietic acid and violamine. 20

ARPAD V. BIEHLER.

CERTIFICATE OF CORRECTION.

Patent No. 1,998,530.

April 23, 1935.

ARPAD von BIEHLER.

It is hereby certified that error appears in the printed specification of the above numbered patent requiring correction as follows: Page 2, first column, line 14, claim 2, for "salts" read solvents; and that the said Letters Patent should be read with this correction therein that the same may conform to the record of the case in the Patent Office.

Signed and sealed this 6th day of August, A. D. 1935.

(Seal)

Leslie Frazer  
Acting Commissioner of Patents.